

## UNITED STATES PATENT OFFICE.

JOHN F. MYERS, OF NEW YORK, N. Y.

## POLISH.

SPECIFICATION forming part of Letters Patent No. 733,591, dated July 14, 1903.

Application filed May 2, 1903. Serial No. 155,414. (No specimens.)

*To all whom it may concern:*

Be it known that I, JOHN F. MYERS, a citizen of the United States, residing at New York, New York county, New York State, 5 have invented certain new and useful Improvements in Polishes, of which the following is a full, clear, and exact description.

My invention relates to polishes, more particularly to stove-polishes.

10 It is the object of my invention to provide a polish which is non-inflammable and non-explosive. Such a polish may be used with entire safety at all times.

Heretofore polishes of a liquid or pasty 15 form have included inflammable or explosive ingredients, which have rendered them dangerous to manufacture, store, or use.

My improved polish consists, essentially, 20 of a base composed of a graphite, plumbago, or other suitable mineral product, which is mixed with tetrachlorid of carbon, the same acting as a vehicle for the same. It will thus be apparent that this agent aids in conveying said base to its intended destination—for example, the outside of a stove or other metallic 25 surface that it is desired to polish. After the polish is applied the tetrachlorid of carbon, being exposed to the air, will evaporate and leave the base in a thin layer over the surface

30 to which it has been applied. After this the said coating may be rubbed down and polished in the usual way by a cloth or brush. By employing tetrachlorid of carbon as a vehicle for the polish I am also permitted to utilize benzin 35 in the mixture without danger. I prefer to use benzin as one of the ingredients, since I have found that superior results are attained. To that end I have mixed with the liquefying agent as much as twenty per cent. of benzin

40 of 62° Baumé without securing a product which will give off gases of an inflammable or explosive nature. While I have spoken of twenty per cent. of benzin as being the quantity that I have employed, I do not mean that

45 it need not be more or less nor do I mean that the presence of benzin is essential. Included in this mixture I also preferably use a coloring-matter—for example, carbon-black or the like—and also an adhesive agent—for example, varnish—the function of the former being

50 to give to the base a decidedly black coloring, the function of the latter being to cause the base to cling tenaciously to the surface to which the polish is applied. These ingredients are added in such proportions as are well known to the mechanic skilled in the art of 55 making polishes.

One example of a formula for making a 60 polish for stoves or other metal surfaces, in which I employ all of these different ingredients, is as follows: Thirty pounds of graphite or plumbago, five pounds of carbon-black, five pounds of varnish, adding any desired amount of a liquid vehicle to reduce said solids to the desired liquid or pasty state, 65 said liquid being composed of eighty per cent. tetrachlorid of carbon and twenty per cent. of benzin of 62° Baumé. These different ingredients when mixed together and agitated assume a consistency depending upon the 70 quantity of the liquid employed. Hence the polish may be marketed either in the form of paste or in the form of a liquid, according to the desires of the manufacturer or user.

I have found that the tetrachlorid of carbon 75 neutralizes the inflammable and explosive qualities of the benzin, so that the polish may be manufactured, stored, or used with entire safety.

While I have spoken of benzin as an element of the liquid agent, it should be understood that other products of petroleum or oils may be substituted, and therefore in using the term "benzin" I intend to include such other products as may be useful in supplementing 85 the tetrachlorid of carbon.

This polish is useful not only in blacking and polishing stoves, but it may be employed in polishing nickel, brass, or other bright work.

90 What I claim is—

1. A polish composed of a mineral base mixed with tetrachlorid of carbon as a vehicle therefor.
2. A polish composed of a mineral base of graphite mixed with tetrachlorid of carbon as a vehicle therefor.
3. A polish composed of a base of graphite mixed with a liquid vehicle composed of tetrachlorid of carbon and a lesser quantity of 95 benzin.
4. A polish composed of a base of graphite 100

mixed with a liquid vehicle containing tetrachlorid of carbon, said polish including also a black coloring-matter.

5. A polish composed of a base of graphite and a liquid vehicle containing tetrachlorid of carbon, a lesser quantity of benzin and an adhesive agent.

6. A polish composed of a mineral base mixed with a non-inflammable and non-explosive chlorid of carbon as a vehicle therefor.

7. A polish composed of a mineral base and a liquid vehicle containing benzin and an agent to neutralize the inflammable and explosive qualities thereof.

Signed at New York, N. Y., this 1st day of 15 May, 1903.

JOHN F. MYERS.

Witnesses:

R. C. MITCHELL,  
L. VREELAND.